

[54] **PROCESS OF MAKING COLD REDUCED STEEL**

[75] Inventors: **Kazuo Matusdo; Takayoshi Shimomura; Kooichi Oosawa, all of Fukuyama, Japan**

[73] Assignee: **Nippon Kokan Kabushiki Kaisha Chiyoda-ku, Tokyo, Japan**

[22] Filed: **Jan. 25, 1971**

[21] Appl. No.: **109,446**

[30] **Foreign Application Priority Data**

Feb. 2, 1970 Japan ..... 45-8451

[52] U.S. Cl. ..... 148/12.1, 148/12 C

[51] Int. Cl. ..... C21d 9/48

[58] Field of Search ..... 148/12, 12.1

[56] **References Cited**

UNITED STATES PATENTS

3,178,318 4/1965 Shimizu et al. ..... 148/12

|           |         |                     |          |
|-----------|---------|---------------------|----------|
| 3,215,567 | 11/1965 | Yoshida .....       | 148/12   |
| 3,239,390 | 3/1966  | Matsukura .....     | 148/12.1 |
| 3,248,270 | 4/1966  | Laidman et al. .... | 148/12   |
| 3,264,144 | 8/1966  | Frazier et al. .... | 148/12   |

Primary Examiner—W. Stallard  
Attorney, Agent, or Firm—Ulle C. Linton

[57] **ABSTRACT**

A making process of cold reduced steel, which is specially produced by continuous annealing line, characterized by making ingot that carbon is from 0.03% to 0.06% and oxygen is from 0.05% to 0.10%, decarburizing the hot strip at temperature of less than 780°C, and finally annealing said strip at temperature of more than recrystallization temperature to  $A_3$  point.

4 Claims, 1 Drawing Figure



PATENTED FEB 11 1975

3,865,637



INVENTORS  
KAZUO MATSUDO, TAKAYOSHI SHIMOMURA,  
AND KOOICHI OOSAWA  
BY

*Linton and Linton*  
ATTORNEYS

## PROCESS OF MAKING COLD REDUCED STEEL

This invention relates to an improved process of making cold reduced steel having good press formability which is specially possible to be produced in large scale by continuous annealing line.

It is well known that there are many papers or patents in the field of deep drawable steel making, which is by means of adjusting chemical composition in steel, setting up rolling condition of the steel, and/or controlling heat treatment of the steel. These processes are commonly employed to make good drawable steel and very effective in making said steel. It is, however, a fact that there is a limit of itself in said drawability of ordinary rimmed steel, even though the known decarburization annealing process is added to the final stage. That is, the above decarburization annealing process have a tendency to make crystal grain coarse and result in bringing about known orange peel on surface of the steel in press forming stage. We inventors' experiments show that steel should be annealed at temperature of about 700°C in order to avoid such phenomenon. It will be impossible to improve said drawability of the steel.

This invention is developed to improve the above fault and to make the effect of said decarburizing process demonstrate fully. The features of this invention lie in decarburizing hot strip before cold reducing of the strip. How to treat the decarburized hot strip is sufficient to depend on ordinary steps, which is cold-reduced, box-annealed or passed through continuous annealing line and then temper-rolled. Press formability of said strip treated with the above steps is far better than that of the common process.

Thus, an object of this invention is to provide an improved process of making cold reduced steel having for more excellent press formability than that of the steel produced by conventional process.

Another object of this invention is to provide an improved process of making cold reduced steel being capable to demonstrate good drawability even in the case of being treated with common continuous annealing line.

Other objects and advantages will be apparent with the following detailed description and by the accompanying drawing in which:

The accompanying drawing shows interrelation and amount of oxygen in rimmed steel, which have direct effects upon ferrite grain.

In this invention, low carbon rimmed steel ingot should be made within the range of 0.03% to 0.06% carbon and 0.05% to 0.10% oxygen in steel making furnace. The hot strip, which is rolled from the above ingot, is decarburized at less than 780°C temperature and then is cold-reduced in the ordinary manner. Such a cold-reduced strip is finally annealed at a temperature of less than  $A_3$  point to more than recrystallization temperature of the steel and then is temper-rolled.

In the above process, the reason that said carbon content is limited to the range of 0.03% to 0.06% is as follows: less than 0.03% carbon is impossible to be made with the ordinary steel making process, and more than 0.06% carbon is difficult to be effectively decarburized. The reason that said oxygen content is limited to the range of 0.05% to 0.10% lies in that less than 0.05% oxygen causes said ferrite grain to coarsen, and more than 0.10% oxygen gives a great damage to cleanliness of the steel. The interrelation between the above

oxygen content and decarburization temperature is the most important factor in this invention. The accompanying drawing shows the results of the above interrelation, which is obtained by many experiments.

- 5 Referring now to said drawing, it is possible to be well understood that the scope that uniform grain is possible to be obtained is the region enclosed by oxygen content of more than 0.05% and decarburization temperature of less than 780°C. However, the region of more than 10 0.06% oxygen and less than 750°C should be recommended as the most preferable scope. The scope of less than 0.05% oxygen and more than 770°C decarburization temperature is scarcely employed, because it is confirmed as the region of coarsening grain. This is the reason that decarburization temperature is limited to less than 780°C. Such a decarburizing annealing is carried out with common open coil annealing furnace.
- 15 The strip after cold reducing is annealed at a temperature of more than recrystallization temperature to less than  $A_3$  point. Such a final annealing can be put into practice with either box type annealing furnace of continuous annealing furnace. It is, in the case of the latter, confirmed that there is shown many advantages in comparison with the common continuous annealing process. Firstly, the mechanical properties of this invention steel is far better than that of the steel produced by common continuous annealing process, as mentioned later. Secondly, while decarburization annealing in this invention is carried out for hot rolled strip, solution carbon in ferrite becomes very low, consequently aging resistibility of the steel is possible to be improved. Thirdly, in this invention, the annealing temperature near  $A_3$  point is possible to be employed as mentioned later. Even though such a high temperature, there is no coarsening of recrystallized grain. This is a large advantage and a great improvement of mechanical properties is obtained. It is needless to say that the same effect as mentioned above will be obtained in the case of said box type annealing.
- 20
- 25
- 30
- 35
- 40

Actual example of this invention process are as follows:

## EXAMPLE I

45 Steel making furnace: LD convertor

Chemical composition: as in Table I

Table I

|    |                                                                                                                                                                                            |                                                                                                                                  |
|----|--------------------------------------------------------------------------------------------------------------------------------------------------------------------------------------------|----------------------------------------------------------------------------------------------------------------------------------|
| 50 | C: 0.05<br>Mn: 0.33<br>P: 0.011<br>S: 0.017<br>N: 0.0016<br>O: 0.058                                                                                                                       | Hot rolling condition after slabbing:<br>finishing temperature: 850°C<br>coiling temperature: 595°C<br>thickness of strip: 2.3mm |
| 55 | Decarburizing condition after pickling:<br>employed annealing furnace:<br>atmosphere: wet hydrogen<br>soaking temperature: 730°C × 10hr.                                                   | open coil furnace<br>wet hydrogen<br>730°C × 10hr.                                                                               |
| 60 | carbon in steel:<br>Cold reducing condition:<br>reducing ratio:<br>thickness of strip:<br>Final annealing condition:<br>employed furnace:<br>soaking temperature:<br>Temper rolling ratio: | 0.003%<br>73.9%<br>0.6mm<br>ordinary continuous annealing furnace<br>700°C × 1 min.<br>1.5%                                      |

The mechanical properties of the above mentioned steel is shown in Table II.

Table II

|                                         |      |
|-----------------------------------------|------|
| Yield point (Kg/mm <sup>2</sup> ):      | 18.4 |
| Elongation of yield point (%):          | 0    |
| Tensile strength (Kg/mm <sup>2</sup> ): | 29.3 |
| Total elongation (%):                   | 49.8 |
| Lanford value r:                        | 1.56 |
| Aging index (Kg/mm <sup>2</sup> ):      | 5.5  |
| Hardness HR - 30T:                      | 42.8 |

## EXAMPLE II

Producing requirements are the same as those of Example I, except soaking temperature of the continuous annealing.

Soaking temperature: 800°C × 1 min.

The mechanical properties of the above steel is as follows:

Table III

|                                         |      |
|-----------------------------------------|------|
| Yield point (Kg/mm <sup>2</sup> ):      | 17.2 |
| Elongation of yield point (%):          | 0    |
| Tensile strength (Kg/mm <sup>2</sup> ): | 28.6 |
| Total elongation (%):                   | 50.3 |
| Lanford value r:                        | 1.68 |
| Aging index (Kg/mm <sup>2</sup> ):      | 5.2  |
| Hardness HR - 30T:                      | 41.5 |

A steel compared with Example I and II was produced by the ordinary continuous annealing process. That is, the making conditions are the same as those of said Example, except the annealing condition.

Annealing condition:

decarburization: not employed

soaking temperature of continuous annealing process: 700°C × 1 min.

The mechanical properties of the steel is as follows:

Table IV

|                                         |      |
|-----------------------------------------|------|
| Yield point (Kg/mm <sup>2</sup> ):      | 25.5 |
| Elongation of yield point (%):          | 0.7  |
| Tensile strength (Kg/mm <sup>2</sup> ): | 34.8 |
| Total elongation (%):                   | 41.4 |
| Lanford value r:                        | 1.15 |
| Aging index (Kg/mm <sup>2</sup> ):      | 7.3  |
| Hardness HR - 30T:                      | 53.6 |

According to Table IV, it will be understood that the steel is impossible to be employed for press forming. The mechanical properties are too low in comparison with those of Examples I and II of this invention steel.

## EXAMPLE III

This is an example that a box type annealing is employed as the final annealing. The producing conditions are as follows:

Steel making furnace: LD convertor

Chemical composition: as in Table V

Table V

|     |        |
|-----|--------|
| C:  | 0.04   |
| MN: | 0.32   |
| P:  | 0.010  |
| S:  | 0.016  |
| N:  | 0.0017 |
| O:  | 0.061  |

Hot rolling condition after slabbing:

Table V-Continued

|                                         |                                                         |
|-----------------------------------------|---------------------------------------------------------|
| finishing temperature:                  | 850°C                                                   |
| cooling temperature:                    | 590°C                                                   |
| thickness of strip:                     | 2.3mm                                                   |
| Decarburizing condition after pickling: | open coil annealing furnace                             |
| employed furnace:                       | wet hydrogen                                            |
| atmosphere:                             | 730°C × 10hr.                                           |
| soaking temperature:                    | carbon in steel: 0.003%                                 |
| Cold reducing condition:                | 65.2%                                                   |
| reducing ratio:                         | thickness of strip: 0.8mm                               |
| Final annealing condition:              | employed furnace: ordinary tight coil annealing furnace |
| atmosphere:                             | HNX gas                                                 |
| soaking temperature:                    | 700°C × 5hr.                                            |
| Temper rolling ratio:                   | 1.0%                                                    |

The mechanical properties of the above steel are shown in Table VI.

Table VI

|                                         |      |
|-----------------------------------------|------|
| Yield point (Kg/mm <sup>2</sup> ):      | 18.1 |
| Elongation of yield point (%):          | 0    |
| Tensile strength (Kg/mm <sup>2</sup> ): | 28.8 |
| Total elongation (%):                   | 52.1 |
| Lanford value r:                        | 1.84 |
| Aging index (Kg/mm <sup>2</sup> ):      | 4.8  |
| Hardness HR - 30T:                      | 38.1 |

## EXAMPLE IV

Producing requirements are the same as those of Example III, except soaking temperature of the box type annealing,

Soaking temperature: 800°C × 5hr

The mechanical properties of the above steel are as follows:

Table VII

|                                         |      |
|-----------------------------------------|------|
| Yield point (Kg/mm <sup>2</sup> ):      | 16.4 |
| Elongation of yield point (%):          | 0    |
| Tensile strength (Kg/mm <sup>2</sup> ): | 27.9 |
| Total elongation (%):                   | 53.6 |
| Lanford value r:                        | 1.93 |
| Aging index (Kg/mm <sup>2</sup> ):      | 4.9  |
| Hardness HR - 30T:                      | 35.9 |

A steel compared with Examples III and IV was produced by the ordinary box type annealing process. That is, the making conditions are the same as those of said Example, except the annealing condition:

Annealing condition:

decarburization: not employed

soaking temperature of box type annealing process: 700°C × 5hr

The mechanical properties of the steel are as follows:

Table VIII

|                                         |      |
|-----------------------------------------|------|
| Yield point (Kg/mm <sup>2</sup> ):      | 21.9 |
| Elongation of yield point (%):          | 0    |
| Tensile strength (Kg/mm <sup>2</sup> ): | 32.5 |
| Total elongation (%):                   | 47.2 |
| Lanford value r:                        | 1.30 |
| Aging index (Kg/mm <sup>2</sup> ):      | 4.8  |
| Hardness HR - 30T:                      | 46.0 |

According to the above Table VIII, it will be understood that all of the mechanical properties are far lower than those of Example VI and VII.

Thus, it is understood that the process of this invention is making splendid accomplishments. We must not take that it was itself necessary. That is, the first reason lies in the final annealing for the steel that carbon content in steel is very low. The second reason is that said first reason causes growth of recrystallizing grain and make texture of (111) direction greater in occupying rate. Accordingly, press formability of this invention steel is far higher than that of usual steel, even though its grain size is the same as that of another steel.

What is claimed is:

1. An improved process of making cold reduced steel consisting in producing low carbon rimmed steel of 0.03 to 0.06% C and 0.05 to 0.10% O, decarburizing said steel at less than 780°C, cold-reducing said steel,

finally annealing said cold-reduced steel at less than  $A_3$  point to more than recrystallization temperature and then temper-rolling said steel.

2. An improved process of making cold reduced steel set forth in claim 1 wherein the final annealing is continuous annealing.

3. An improved process of making cold reduced steel set forth in claim 1 wherein the final annealing is box type annealing.

4. An improved process of making cold reduced steel set forth in claim 1 wherein the oxygen content is within the range of 0.06 to 0.10% and the decarburizing temperature is less than 750°C.

\* \* \* \* \*

15

20

25

30

35

40

45

50

55

60

65